# EUROPEAN PATENT SPECIFICATION

(11) **EP 3 135 811 B1**
(45) Date of publication and mention of the grant of the patent: **11.10.2017**
(21) Application number: 15182673.2
(22) Date of filing: 27.08.2015
(51) Int. Cl.: D21H 11/12, D21H 13/10, D21H 13/26, D21H 17/51, D21J 1/00, D21C 1/02, D21B 1/16

(54) **PRODUCTION METHOD OF PULP DERIVED FROM BIOMASS FOR PRODUCING COMPOSITE BOARDS**
HERSTELLUNGSVERFAHREN FÜR AUS BIOMASSE GEWONNENEN ZELLSTOFF ZUR HERSTELLUNG VON VERBUNDPLATTEN
PROCÉDÉ DE PRODUCTION DE PÂTE À PAPIER DÉRIVÉE DE BIOMASSE POUR LA PRODUCTION DE PANNEAUX COMPOSITES

(43) Date of publication of application: 01.03.2017
(73) Proprietor: VestaEco SA, 13-230 Lidzbark (PL)
(72) Inventor: KOCEWICZ, Robert, 00-728 Warszawa (PL); DANECKI, Leszek Stanislaw, 89-650 Czersk (PL)
(74) Representative: Markieta, Jaroslaw Franciszek

(56) References cited:
- WO-A1-00/25600
- AT-B- 277 746
- US-A- 5 656 129
- US-A1- 2004 112 557

## Description

The subject of an invention is a production method of pulp for producing composite boards from lignocellulosic fibres derived from biomass, as well as a pulp board produced according to the method.

Boards made from pulp are applied in timber industries, i.e. for producing furniture, floor panels, decorative strips, as well as in the construction sector as insulating materials, both thermal and acoustic.

A demand for cheap construction materials, including boards for furniture production, has led to creating composite materials based on materials (residues) derived from woodworking. An example of such materials that are very well known in industry is a chipboard and a fibreboard. A chipboard is produced through joining relatively large fragments of wood with resin, whereas a fibreboard is produced through connecting separated lignocellulosic fibres with resin.

Materials derived from woodworking became more expensive and less available, which has led to the development of board production on the basis of lignocellulosic fibres of non-wooden origin. A method of chipboard production with the use of resources derived from agriculture, such as straw, is known from US 5,656,129 patent document. Blades are cut, soaked in water and treated with steam under high pressure in order to soften the stems. Blades prepared in such a way may be mixed in any proportions with other fibre materials, such as fibres derived from wood, and used in wet, dry, and wet-dry wood-like board production.

US 6,596,209 document presents a production of chipboards from materials of non-woodworking origin, where resources preferred are selected according to high cellulose and hemicellulose level and low silica level. The processing method is characterized by a short time of cleaning and low pressure of steam softening the blades. Waste derived from agriculture, such as straw of different origin, grass, paper production waste (collectively defined as biomass), is used as a resource.

Traditionally, fibreboards are made from fibres of deciduous or coniferous trees, joined together with waxes or resins in high temperature and increased pressure. Boards produced in such a way are characterized by high homogeneity and dimensional stability, constituting a valued building material. Production parameters have an influence on the end product parameters, such as durability and density, which allows to obtain boards for various purposes. Low density boards are suitable for acoustic insulation, whereas high density boards are used in woodwork.

Properties of fibreboards may exceed parameters of solid wood, and the possibility of using various additives allows to produce boards with special parameters, such as fire resistance and moisture resistance. Using antraquinone known from the paper production process positively influences water resistance of the boards.

Using sodium silicate in wood-like board production generally increases fire resistance; however, it causes the boards to become susceptible to water. In US 4,761,342 document, an inorganic binding additive to boards increasing their fire resistance has been revealed. This additive consists of calcium and/or magnesium, sulphur or inorganic sulphur compound, and alkaline metal silicate. This additive does not contain organic resins, which may emit harmful gases.

US 1,627,103 document reveals a board production processed based on fibres from sugarcane residue boiled in calcium hydroxide solution. Before forming a board, insecticides may be added to fibres treated in such a way in order to produce an insect resistant board. In order to produce a board of increased durability, it is possible to add cement with sodium silicate. A product obtained in such a way may be cut, sawn and processed similarly to ordinary wood.

The publication of US 20030015283 patent application reveals the method of wood-like board production method based on water hyacinth characterized by satisfactory parameters even without using synthetic additives, such as resin. Yet, it is only an exception; various forms of resins and thermoplastic materials are used for joining lignocellulosic fibres in fibreboards.

However, WO 2006076814 patent document reveals urea, melamine, formaldehyde, phenolic and isocyanate resins as fillers joining lignocellulosic fibres in a board. WO2006076814 document reveals potential sources of fibres for producing fibreboards. Fibres suitable for fibreboard production may be derived from widely cultivated plants, such as hemp, sugarcane, bamboo, banana tree stems and leaves, coir, coconut, corn, cotton, flax, papyrus, rice, wheat, rye, grass, straw and oats. Using such materials allows to limit the amount of agricultural waste and save valuable resources such as wood.

EP 0644861 document reveals a method of cellulosic fibre mass production from fragmented waste paper and wood waste, which is formed into boards after mechanical treatment. EP 1412566 reveals a method of producing nonwoven fabric including the use of cellulosic fibres from waste paper processing that are bound with the help of thermoplastic elastomer fibres. Both various kinds of waxes, such as beeswax, paraffin, lanolin and jojoba oil, and plastics, such as polyethylene and polypropylene, are often used as additives.

US 2004/0112557 A1 discloses methods of bleaching mechanical pulp under alkaline conditions with hydrogen peroxide. The methods include introducing a source of magnesium ions and hydroxyl ions to a refiner. The wood particulates are refined into a pulp in the presence of the magnesium ions and hydroxyl ions, and optionally perhydroxyl ions to simultaneously refine and bleach the pulp in a refiner.

With today's technology, using hydrothermal treatment assuming the use of water at high temperature and high pressure has been revealed as the first stage of production of pulp derived from biomass. Using large amounts of water at high temperature, often in the form of superheated steam under high pressure, has a negative influence on the economic balance; it is expensive and energy-intensive.

The essence of the invention is the method of pulp production for producing boards; cereal straw is fragmented to the form of blades with a length from 10 to 50 mm, which are then subjected to hydrothermal treatment. Mass obtained is injected with the help of a feeding machine between the milling plates of the defibering unit until it is defibered, and then pressed with the help of a screw press until obtaining absolute humidity below 50%. Mass obtained is loosened into the pulp form and dried. The method is characterized in that the cut cereal straw blades are subjected to hydrothermal treatment with water mixture at temperature below 50°C, where hydrothermal treatment does not last longer than 1 minute.

Thanks to introducing the method according to the invention, energy consumption of the production process is reduced both by reducing the demand for thermal energy necessary for heating technological water and by reducing electrical energy necessary for conducting the loosening process. Also, a further technological effect is reducing the risk of charring/scorching fibres on round knives in further stages of production.

Also, a method according to the invention is characterized in that a hydrothermal treatment takes place in water and lye solution. Such a solution allows straw maceration and results in reducing energy consumption of the defibering process.

Also, a method according to the invention is characterized in that a hydrothermal treatment takes place while evenly feeding mass of concentration between 8 and 10% between round knives.

Thanks to introducing mass concentration from the range according to the invention an increase of production energy consumption may be avoided when the concentration is below 8%, which results from larger amount of technological water per dry mass unit. Also, reducing concentration to 10% reduces the risk of charring/scorching fibres on round knives and the risk of hampered transport of wet mass in further production stages.

Also, a method according to the invention is characterized in that cellulosic resources, especially waste paper fibres in a proportion up to 50% by weight of cellulosic fibres, are also added to cereal straw blades. Such a solution conveniently influences the cohesion of mass, since cellulosic fibre is finer than straw fibre.

Also, the method according to the invention is characterized in that cereal straw is fragmented to the form of blades with a length from 10 to 50 mm, conveniently to 30 mm. The lengths of fibres according to the invention conveniently influence physical-mechanical properties of products obtained.

An essence of the invention is also a pulp board, characterized in that it contains pulp produced according to the method according to the invention and the binder.

A board according to the invention is characterized in that it also contains an additive of non-defibered particles of lignocellulosic material, amounting from 1% to 50% by weight. Thanks to introducing defibered particles, it is possible to shape physical-mechanical properties of a ready product.

A board according to the invention is characterized in that it also contains an additive of plastic fibres, especially an additive of aramid fibres. Thanks to introducing non-defibered particles, it is possible to shape physical-mechanical properties of a ready product.

A board according to the invention is characterized in that it also contains an additive of cellulosic acetate. Thanks to the introduction of cellulosic acetate, an improvement of hydrophobic properties and cohesion of the boards has been obtained.

A board according to the invention is characterized in that its binder is melamine-urea-formaldehyde resin, isocyanate adhesive or mixture of both, conveniently in the amount relative to dry mass of the product between 5% and 15%, more conveniently between 8% and 12%. Using a binder according to the invention in the proportions indicated above allows to obtain required usage properties (including especially durability) of boards.

The advantage of the invention is using agricultural waste for producing dry-formed boards. Boards of low density may be used as insulation material and as external room insulation, securing i.e. against changes caused by weather conditions. Specific properties of the product allow to protect buildings against overheating in summer and overcooling in winter. Also, the building material of the board is characterized by high capacity of noise suppression, thanks to which the transfer of high pitched sounds from external sources is significantly reduced. The product of medium density constitutes an alternative to MDF, HDF and OSB boards used in the furniture sector, competitive both in quality and price.

Using pulp obtained from straw and waste paper increases the product's resistance to swelling and tensile strength perpendicular to board surface without a negative influence on the remaining properties of boards produced.

A low level of energy is necessary for obtaining a resource, which results in lower production costs and a lower price of an end product.

Using rapidly renewable resources of waste character, both in the form of re-used straw constituting waste from cereal production process and waste paper undergoing recycling process, together with reducing energy consumption and limiting the use of additives with a strong environmental impact (mainly harmful binders) causes the fibreboard as the subject of the invention to be a product almost perfectly suitable for re-processing, thanks to which its influence on the environment is significantly reduced. Composting and biodegradation of low and medium density boards is possible.

An advantage of the method of board production according to the invention is using easily accessible and rapidly renewable materials constituting agricultural waste for producing wood-like boards in the process of resource treatment in lowered temperature. Mass obtained in such a way is characterized by a specific amount of fats and other hydrophobic substances. Mass obtained in such a way may be stored in a silo for further use or directly mixed with resin and additives, and fed to the board production press. Thanks to natural occurrence of hydrophobic substances in straw, such a board is characterized by an increased moisture resistance.

The subject of the invention has been presented in more detail in a convenient example of execution in a form of a drawing (fig. 1), in which the process of pulp production and pulp board has been schematically shown.

Fig. 1 presents the process of pulp production and its further treatment in order to produce a wood-like board. At the beginning, resources are cleaned in order to remove small stones and other non-organic materials. Next, cereal straw with additives is fragmented until obtaining fibres with a length from 30 to 50 m. Lignocellulosic fibres cut in such a way are loosened hydrothermally in temperature of 50°C. Water and lye solution is fed into the zone between the milling plates. The resource is loosed mechanically through injecting mass with the help of a feeding machine between the milling plates zone of an appropriate defibering unit, while water is fed simultaneously to the milling zone in order to remove excess heat released in the defibering process. After short-time defibering, mass is pressed with the help of a screw press until obtaining humidity below 50%, and loosened with a mixer and dried into the dry fibre mixture form. Mass obtained in such a way may be stored in a silo for further use or directly mixed with resin and additives, and fed to the composite board production press.

In a convenient example of execution, biomass used may be derived from agricultural waste, especially straw. Pulp may contain additives in the form of fibres from fragmented waste paper. Straw is fragmented to the form of blades with a length from 10 to 50 mm, which are then subjected conveniently to intense and short hydrothermal treatment with using alkaline solution at temperature lower than 50°C together with an additive of other lignocellulosic resources. The resource is loosed mechanically through injecting mass with the help of a feeding machine between the milling plates zone of an appropriate defibering unit, and pressed with the help of a screw press until obtaining humidity below 50%. Next, mass obtained is loosened into the pulp form and dried. A hydrothermal treatment takes place water and lye solution. A hydrothermal treatment takes place while evenly feeding mass of concentration between 8 and 10% between round knives.

A pulp board may contain an additive of non-defibered particles of lignocellulosic material, amounting from 1% to 50% by weight. A pulp board may also contain an additive of plastic fibres, especially an additive of aramid fibres. A pulp board may contain an additive of cellulosic acetate. A pulp board, the binder of which is melamine-urea-formaldehyde resin or isocyanate adhesive, conveniently in the amount relative to dry mass of the product between 5% and 15%, more conveniently between 8% and 12%.

### Example 1

In the first example, a board made from pulp of low density with using 75% of lignocellulosic fibre and 25% of cellulosic fibre from waste paper has been obtained; the mixture was subjected to treatment method according to the invention, especially with using hydrothermal treatment with water mixture at 50°C. Melamine-urea-formaldehyde resin (MUF) amounting to 10%, together with isocyanate adhesive (pMDI) amounting to 2% relative to dry mass of the product, were used as binders for board production. 10 ppm of nanosilver particles were used as a biocidal additive.

An appropriate time of pressing allows to obtain a board of density from 120 to 300 kg/m³; especially convenient insulation properties are obtained with density from 170 to 190 kg/m³.

### Example 2

In the second example, a board made from pulp of high density with using 70% of lignocellulosic fibre and 30% of cellulosic fibre from waste paper has been obtained; the mixture was subjected to treatment method according to the invention, especially with using hydrothermal treatment with water mixture at temperature of 45°C. Melamine-urea-formaldehyde resin (MUF) amounting to 12% was used as a binder for board production.

An appropriate time of pressing allows to obtain a board of density from 700 to 900 kg/m³; especially convenient mechanical properties are obtained with density from 700 to 750 kg/m³.

## Claims

1. Method of pulp production for producing boards where
cereal straw is fragmented to the form of blades with a length from 10 to 50 mm,
which are subjected to hydrothermal treatment, then
mass obtained in such a way is injected with the help of a feeding machine between the milling plates of the defibering unit, and pressed
with the help of a screw press until obtaining absolute humidity below 50%, then mass obtained is loosened into the pulp form and dried
**characterized in that**
cut cereal straw blades are subjected to hydrothermal treatment with the use of water mixture at temperature below 50°C, where
hydrothermal treatment does not last longer than 1 minute.

2. A method according to claim 1, **characterized in that** a hydrothermal treatment takes place in water and lye solution.

3. A method according to claim 1 and 2, **characterized in that** a hydrothermal treatment takes place while evenly feeding mass of concentration from 8 to 10% between round knives.

4. A method according to any of claims 1-3, **characterized in that** cellulosic resources, especially waste paper fibres in a proportion up to 50% by weight of cellulosic fibres, are also added to cereal straw blades.

5. A method according to any of claims 1-4, **characterized in that** cereal straw is fragmented to the form of blades with a length from 10 to 50 mm, conveniently to 30 mm.

## Patentansprüche

1. Verfahren zur Produktion der Pulpe für Faserplattenproduktion, wo
Getreidestroh zum Plättchenform 10 bis 50 mm lang zerteilt werden,
welche hydrothermal behandelt werden und
die dermaßen erhaltene Masse mithilfe Einspeisemaschine zwischen Mahlplatten der Entfaserungsanlage und
anhand Schraubenspindelpresse eingepresst wird, bis absolute Feuchtigkeit unter 50% erhalten wird,
des Weiteren die erhaltene Masse in die Pulpe ausgelöst und ausgetrocknet wird,
**dadurch gekennzeichnet, dass**
die geschnittenen Strohplättchen einer Hydrothermalbehandlung mit der Wassermischung bei Temperatur unter 50°C ausgesetzt werden, wobei
die Hydrothermalbehandlung nicht länger als 1 Minute dauert.

2. Verfahren nach Anspruch 1, **dadurch gekennzeichnet, dass** die Hydrothermalbehandlung in Wasserlaugenlösung stattfindet.

3. Verfahren nach Anspruch 1 und 2, **dadurch gekennzeichnet, dass** die Hydrothermalbehandlung stattfindet, während die Glatteinspeisungsmasse von 8 bis 10% Konzentration zwischen Rundscheibenmessern zugegeben wird.

4. Verfahren nach Anspruch 1 bis 3, **dadurch gekennzeichnet, dass** der Zellfaserstoff, insbesondere Papierabfallfaser, im Verhältnis bis zum 50% der Zellfaserstoffwage, auch den Getreidestrohplättchen zugegeben wird.

5. Verfahren nach jeglichen Ansprüchen 1 bis 4, **dadurch gekennzeichnet, dass** das Getreidestroh plättchenförmig 10 bis 50 mm geschnitten werden, permissiv bis 30 mm.

## Revendications

1. Procédé de production de pâte à papier pour la production de carton dans lequel
la paille de céréales est fragmentée en forme de lamelles d'une longueur de 10 à 50 mm, qui sont soumises à un traitement hydrothermique, puis
la substance obtenue de cette manière est injectée à l'aide d'une machine d'alimentation entre les plaques de broyage de l'unité défibreuse, et pressée
à l'aide d'une presse à vis jusqu'à l'obtention d'une humidité absolue d'une valeur inférieure à 50 %, puis
la substance obtenue est détachée sous la forme de pâte à papier et séchée
**caractérisé en ce que**
les lamelles découpées en paille de céréales sont soumises à un traitement hydrothermique par l'utilisation d'un mélange d'eau à une température inférieure à 50 °C, où
le traitement hydrothermique ne dure pas plus d'1 minute.

2. Un procédé selon la revendication 1, **caractérisé en ce qu'**un traitement hydrothermique se déroule dans une solution d'eau et de soude.

3. Un procédé selon la revendication 1 et 2, **caractérisé en ce qu'**un traitement hydrothermique se déroule en alimentant de manière régulière la substance d'une concentration de 8 à 10 % entre les lames arrondies.

4. Un procédé selon l'une quelconque des revendications 1 à 3, **caractérisé en ce que** les ressources cellulosiques, particulièrement les fibres de déchets de papier dans une proportion allant jusqu'à 50 % du poids des fibres cellulosiques, sont également ajoutées aux lamelles en paille de céréales.

5. Un procédé selon l'une quelconque des revendications 1 à 3, **caractérisé en ce que** les pailles de céréales sont fragmentées sous forme de lamelles d'une longueur allant de 10 à 50 mm, idéalement de 30 mm.
